

## UNITED STATES PATENT OFFICE.

RUSSELL GEORGE PELLY, OF LONDON, ENGLAND, ASSIGNOR TO TECHNICAL RESEARCH WORKS, LIMITED, OF LONDON, ENGLAND.

## LUBRICANT AND PROCESS OF PREPARING SAME.

No Drawing.

Application filed September 29, 1922. Serial No. 591,420.

To all whom it may concern:

Be it known that I, RUSSELL GEORGE PELLY, a subject of the King of Great Britain, and resident of London, England, have **5** invented a certain new and useful Lubricant and Process of Preparing Same, of which the following is a specification.

This invention relates to an improved process for increasing the lubricating properties of oils. Admixtures of saponifiable **10** oils, fats or waxes with mineral hydrocarbon oils (compounded oils) have been employed as lubricants to a large extent, it being well known that mineral hydrocarbon **15** oils are not so efficient for use as lubricants in many cases as saponifiable oils, fats or waxes of animal or vegetable origin.

For the purpose of carrying out my invention I add to mineral oils or to saponifiable **20** oils, fats, or waxes derivatives of aliphatic polyhydric alcohols or phenols in which the hydroxyl groups are partially replaced by fatty and/or other acid radicles, for example the monoglycerides of such fatty acids **25** as oleic or lauric acid, which results in the production of a lubricating oil of greater efficiency and by the selection of substances of the nature mentioned valuable properties, such as the stiffening of the consistency and **30** the emulsification with aqueous liquids may be imparted to saponifiable or mineral oils.

For example I have found that the addition of five per cent of mono- or di-glyceride of oleic acid to an ordinary mineral lubricating oil reduces the co-efficient of friction **35**

and improves its emulsifying property in water.

The compounds which have been found to give the best results in my invention are the mono- and diglycerides of the common fatty **40** acids (for example, oleic, lauric or stearic acids); in other words, a polyhydric alcohol, viz; glycerol in which the (OH) groups are partially replaced by acids radical; their preparation is best effected by the method **45** described in Brit. Pat. 163,352 "An improved process for the conversion of fatty acids or oils or fats containing free fatty acids into glycerides," by E. R. Bolton and E. J. Lush (the property of Technical Re- **50** search Works Limited).

What I claim is:—

1. That method of increasing the lubricating properties of oils which consists in adding to said oils the derivatives of aliphatic **55** polyhydric alcohols formed by partially replacing the hydroxyl groups by acid radicals.

2. A composition of matter consisting of lubricating oil and aliphatic polyhydric alcohols of which the hydroxyl groups are partially replaced by acid radicals, substantially as described. **60**

3. A composition of matter consisting of lubricating oils and aliphatic polyhydric alcohols of which one (OH) group is partially replaced by an acid radical forming a monoglyceride, substantially as described. **65**

In testimony whereof I affix my signature.

RUSSELL GEORGE PELLY.